# EUROPEAN PATENT SPECIFICATION

(11) **EP 2 367 637 B1**
(45) Date of publication and mention of the grant of the patent: **08.05.2019**
(21) Application number: 09835791.6
(22) Date of filing: 22.12.2009
(51) Int. Cl.: B05D 1/14, B05D 1/16, B32B 33/00, D06Q 1/12, D06Q 1/00, D06Q 1/14

(54) **APPLYING A DESIGN ON A TEXTILE**
AUFBRINGUNG EINES DESIGNS AUF EINEM STOFF
APPLICATION D'UN DESSIN SUR UNE ÉTOFFE

(30) Priority: 22.12.2008 IE 20081016; 12.01.2009 US 143992 P; 22.12.2009 US 644725
(43) Date of publication of application: 28.09.2011
(73) Proprietor: Illinois Tool Works Inc., Glenview, IL 60025 (US)
(72) Inventor: CREMIN, Celine, M., County Cork (IE); MOLONEY, Padraig, M., County Cork (IE)
(74) Representative: HGF Limited
(86) International application number: PCT/US2009/069277
(87) International publication number: WO 2010/075436

(56) References cited:
- WO-A1-2008/049030
- WO-A2-2004/005415
- US-A- 5 207 851
- US-A- 5 240 587
- US-A- 5 655 458
- US-A- 5 855 980
- US-A- 5 914 176
- US-A- 6 083 332
- US-A- 6 110 560
- US-A1- 2005 266 204
- US-A1- 2008 095 973
- US-A1- 2008 302 772
- US-B2- 7 410 682
- US-B2- 7 465 485

## Description

### BACKGROUND OF THE INVENTION

The invention relates to application of designs to textiles.

GB2245220 describes a multi-layer transfer sheet, in which granules are fixed to a permanent adhesive layer on flock fibres. To apply the design to a textile, the granule layer is placed against the textile surface and heat and pressure are applied. The granules melt and seep into the fabric to fix the design, and a disposable peel-off sheet is peeled away. GB2245220 involves a large number of processing steps, which include multiple drying and screen printing operations. With this process there are potentially issues of coverage over certain colours and durability on certain types of fabric.

Accordingly, there is a need for improved application of designs to textiles, in terms of versatility in the colour of designs, and/or ease of application, and/or durability, and/or resistance to dye migration into the textile. Such an improved application also reduces manufacturing operations and provides an ability to use any of a variety of raw materials such as: woven textiles, hot-melt films, and/or flocking adhesive. Other objectives are to achieve greater flexibility, durability and/or resistance to dye migration.

US2008/0095973A1 describes a flocked article and method for forming the flocked article.

US2008/0302772A1 describes a process for laser-cutting a pattern for decorating textile articles.

US5207851 describes a combination flock and other material transfer.

US7410682B2 describes a flocked stretchable design and a process for producing a flocked stretchable design.

### BRIEF SUMMARY OF THE INVENTION

An applique for applying a design to a fabric includes a flock in a pre-determined multi-colour pattern retained by a flock adhesive and an application adhesive suitable for adhering the applique to a fabric.

In one embodiment, the flock adhesive is deposited on a substrate such as a film or a fabric. In one embodiment, the substrate has multiple colours, viewable in-between the flock. In one embodiment, the substrate is of polyurethane material. Alternately, the substrate is of fabric material. The fabric material can be sublimated with a pre-printed pattern. The fabric can be of woven fibre, such as a high-lustre type. The fibre can be a satin or satin-like material. The fibre can be polyester.

The substrate can be a foil material. The foil can include a holographic pattern. The substrate can include a migration-resistant barrier.

The application adhesive can be a hot-melt. A garment or piece of fabric can be provided with the applique as described above.

A method of decorating a garment or piece of fabric includes applying the applique as described above to the fabric using the application adhesive.

For purposes of the present disclosure, the term "applique" means a decorative patch or badge which is applied to a fabric to impart a decorative design such as a logo on the fabric such as a garment.

These and other features and advantages of the present invention will be apparent from the following detailed description, in conjunction with the appended claims.

### BRIEF DESCRIPTION OF THE SEVERAL VIEWS OF THE DRAWINGS

The benefits and advantages of the present invention will become more readily apparent to those of ordinary skill in the relevant art after reviewing the following detailed description and accompanying drawings, wherein:
Fig. 1 is a cross-sectional view of an applique of the invention for application of a design to a garment;
Fig. 2 shows the applique after application onto textile fabric; and
Figs. 3 to 7 are cross-section views of alternative appliques of the invention.

### DETAILED DESCRIPTION OF THE INVENTION

While the present invention is susceptible of embodiment in various forms, there is shown in the drawings and will hereinafter be described a presently preferred embodiment with the understanding that the present disclosure is to be considered an exemplification of the invention and is not intended to limit the invention to the specific embodiment illustrated.

It should be further understood that the title of this section of this specification, namely, "Detailed Description Of The Invention", relates to a requirement of the United States Patent Office, and does not imply, nor should be inferred to limit the subject matter disclosed herein.

Referring to Figs. 1 and 2, an applique 9 in accordance with the principle of the present invention includes a polyurethane ("PU") film 1 onto which a flock adhesive, namely a permanent adhesive layer 2, is printed. As set forth above, for purposes of the present disclosure, the term "applique" means a decorative patch or badge which is applied to a fabric to impart a decorative design such as a logo on the fabric such as a garment.

A flock fibre layer 3 is applied onto the adhesive layer 2 using an electrostatic field. The flock layer 3 can be multi-coloured, in which case, each colour is applied sequentially using a conventional flocking method. An application adhesive, namely a hot-melt layer 4, is laminated to the PU film 1 prior to or after the flocking operations.

The hot-melt adhesive comprises a thermoplastic film made from aromatic or aliphatic thermoplastic. The hot-melt film can include one or more of, but is not limited to, polyamide; polyester; polyolefin; polyurethane; and polyurethane ester. For example, the hot-melt film can be 76 micron Bemis Polyester Hotmelt Film 5250.

To apply a design to a textile, including, for example (but not limited to a satin or satin-like material), the applique 9 is simply placed on the textile after removing the disposable carrier 5, with the hotmelt film 4 in contact with the textile. Heat and pressure are applied so the hot-melt impregnates into the fabric (F) to seal the applique in place. Alternatively, application can be carried out using a high frequency welding method.

The invention has a major advantage of not requiring deposition of any material onto the flock - thus preserving clarity of colour and edge definition of the design. Also, it is very simple to apply, and high-frequency welding or heat and pressure may be used. The invention has the major advantage that the flock fibres are not deposited into a release adhesive which at application will tend to pull out quantities of flock fibres resulting in incomplete flock coverage. The invention makes use of a non-toxic permanent hot-melt adhesive. The cross-linking of the adhesive is one-step and permanent, not requiring additional curing time during application onto the textile. The use of textile films or hot-melt adhesive films also improves the coverage and opacity. Replacing the traditional screen-printing process of the application adhesive (which can be inconsistent in quality) by using films also substantially reduces the risk of waste material.

Referring to Fig. 3, in another embodiment, a multi-colour flock 10 is retained by permanent adhesive 11, which is deposited directly onto hot-melt 12 supplied on a carrier 13. This is a simpler arrangement, avoiding need for a PU or other film substrate. Need for a film is avoided, which allows creation of a very lightweight and potentially very elastic applique. In this embodiment, there is little risk of underlying colours being visible. Referring to Fig. 3, in another embodiment, a multi-color flock 10 is retained by permanent adhesive 11, which is deposited directly onto an opaque hot-melt 12 supplied on a carrier 13. In this embodiment, there is little risk of underlying colors being visible.

Referring to Fig. 4, a multi-colour flock 20 is retained by permanent adhesive 21, which is deposited on a textile 22. Again, there is hot-melt 23 and a carrier 24. This has the advantages of creating a multi-textured and three dimensional applique, the surface of which includes high pile flock fibres and textile satin materials of various textures.

Referring to Fig. 5, in another embodiment, a multi-colour flock 30 is retained by permanent adhesive 31 onto a textile 32 which has been sublimation printed before flocking. The sublimation textile satin material used can be for example of the type supplied by the Company Houlaisha Co. Ltd. in Japan under the name NXSS. This material is disclosed in European patent application EP1876288.

Referring to Fig. 6, a multi-colour flock 40 is retained by adhesive 41 deposited on foil 42, which can be a metallic or reflective or holographic foil. Again, there is hot-melt 43 and a disposable carrier 44. This embodiment of the invention has the advantage of creating multi-textured and three-dimensional appliques into which an element of security, brand protection and authentication can be built in.

Referring to Fig. 7, in another embodiment, a multi-colour flock 50 is retained by adhesive 51, which is deposited on a migration-resistant barrier 52, which can be a single layer or composite migration resistant barrier or membrane layer over hot-melt 53 and a disposable carrier 54 (optional). This embodiment can be used specifically where a high degree of migration/bleed through resistance is required.

The flock adhesives 2, 11, 21, 31, 41, and 51 referred to above are all of the cross-linking water-based acrylic emulsion type, the particular cross-linking for each adhesive being chosen to suit the substrate. While alternatives are possible such as a polyurethane-based adhesive for the adhesive 2 (on PU film), it is believed that water-based acrylic emulsions are more effective and are safer.

The following are examples of the adhesives which can be used in some embodiments.
Adhesive 2 (on PU film 1): Product: TUBVINYL TTH-ZP WEISS, Chemical Description: Acrylate dispersion containing titanium dioxide.
Adhesive 11 (on hot-melt 12): Product: TUBVINYL TTH-ZP WEISS, Chemical Description: Acrylate dispersion containing titanium dioxide.
Adhesive 21 (on textile 22): Product: TUBITRANS BOND-3, Chemical Description: Acrylic Co-Polymer in aqueous dispersion.
Adhesive 31 (on sublimated satin 32): Product: TUBITRANS BOND-3, Chemical Description: Acrylic Co-Polymer in aqueous dispersion.
Adhesive 41 (on foil 42): Product: TUBVINYL TTH-ZP WEISS, Chemical Description: Acrylate dispersion containing titanium dioxide.
Adhesive 51 (on migration-resistant barrier substrate 52): Product: TUBVINYL TTH-ZP WEISS, Chemical Description: Acrylate dispersion containing titanium dioxide. The above adhesives are available from CHT R. BEITLICH GMBH, Werk Oyten, Rudolf-Diesel-StraBe 19-21 28876 Oyten, Germany.

It will be appreciated that the present invention achieves improved application of designs to textiles, including, for example, satin and satin-like materials, in terms of versatility in the colour of designs, and/or ease of application, and/or durability, and/or resistance to dye migration into the textile. The present invention also facilitated reduced manufacturing operations and improves the ability to use any of a variety of raw materials such as woven textiles, hot-melt films, and/or flocking adhesive. This promotes greater flexibility, durability and/or resistance to dye migration.

In the present disclosure, the words "a" or "an" are to be taken to include both the singular and the plural. Conversely, any reference to plural items shall, where appropriate, include the singular.

From the foregoing it will be observed that numerous modifications and variations can be effectuated without departing from the scope of the novel concepts of the present invention. It is to be understood that no limitation with respect to the specific embodiments illustrated is intended or should be inferred. The disclosure is intended to cover by the appended claims all such modifications as fall within the scope of the claims.

## Claims

1. An applique (9) for applying a design to a fabric, the applique comprising:
a substrate (1; 12; 22; 32; 42; 52) comprising polyurethane material, wherein the substrate includes a migration-resistant barrier;
a flock (3; 10; 20; 30; 40; 50) in a pre-determined multi-colour pattern, the flock having fibres;
a flock adhesive (2; 11; 21; 31; 41; 51) securing the flock fibers to the substrate, the flock adhesive being printed on the substrate;
an application adhesive (4; 23; 33; 43; 53), adjacent to the substrate opposite the flock fibers, suitable for adhering the applique to a fabric; and
a carrier layer (5; 13; 24; 44; 54),
wherein the substrate, flock adhesive, and application adhesive are positioned between the flock and the carrier layer and,
wherein the applique is formed without flock being deposited onto a release adhesive.

2. The applique (9) in accordance with claim 1, wherein the substrate (1; 12; 22; 32; 42; 52) has multiple colours, viewable in-between the flock (3; 10; 20; 30; 40; 50).

3. The applique (9) in accordance with claim 1, wherein the substrate (1; 12; 22; 32; 42; 52) is a film.

4. The applique (9) in accordance with claim 3, wherein the film includes a holographic pattern.

5. The applique (9) in accordance with claim 1, wherein the application adhesive (4; 23; 33; 43; 53) is a hot-melt.

6. A garment or piece of fabric (F) comprising an applique (9) in accordance with claim 1.

7. A method of making an appliqué (9) comprising the steps of:
providing a substrate (1; 12; 22; 32; 42; 52) comprising polyurethane material and having a first side and a second side, wherein the substrate includes a migration-resistant barrier;
printing a flock adhesive layer (2; 11; 21; 31; 41; 51) to the first side of the substrate;
applying a flock layer (3; 10; 20; 30; 40; 50 in a pre-determined multi-colour pattern to the flock adhesive layer, the flock having fibres;
securing the flock fibers to the flock adhesive layer;
laminating an adhesive layer (4; 23; 33; 43; 53) on a second side of the substrate; and
providing a selectively removable carrier layer (5; 13; 24; 44; 54) having a side facing the second side of the substrate and another side,
wherein the appliqué is formed without flock being deposited onto a release adhesive.

8. The method in accordance with claim 7 including the step of applying the adhesive layer to a textile (F).

## Patentansprüche

1. Applikation (9) zum Aufbringen eines Designs auf einen Stoff, wobei die Applikation umfasst:
ein Substrat (1; 12; 22; 32; 42; 52), umfassend Polyurethanmaterial, wobei das Substrat eine migrationsbeständige Barriere enthält;
einen Flock (3; 10; 20; 30; 40; 50) in einem vorbestimmten mehrfarbigen Muster, wobei der Flock Fasern aufweist;
einen Flock-Klebstoff (2; 11; 21; 31; 41; 51), der die Flockfasern an dem Substrat fixiert, wobei der Flock-Klebstoff auf das Substrat gedruckt wird;
einen Applikationsklebstoff (4; 23; 33; 43; 53), benachbart zu dem Substrat gegenüber den Flockfasern, der zum Aufkleben der Applikation auf einen Stoff geeignet ist; und
eine Trägerschicht (5; 13; 24; 44; 54),
wobei das Substrat, der Flock-Klebstoff und der Applikationsklebstoff zwischen dem Flock und der Trägerschicht angeordnet sind, und,
wobei die Applikation gebildet wird, ohne dass Flock auf einen ablösbarer Klebstoff abgeschieden wird.

2. Applikation (9) nach Anspruch 1, wobei das Substrat (1; 12; 22; 32; 42; 52) mehrere Farben aufweist, die zwischen dem Flock (3; 10; 20; 30; 40; 50) zu sehen sind.

3. Applikation (9) nach Anspruch 1, wobei das Substrat (1; 12; 22; 32; 42; 52) ein Film ist.

4. Applikation (9) nach Anspruch 3, wobei der Film ein holographisches Muster enthält.

5. Applikation (9) nach Anspruch 1, wobei der Applikationsklebstoff (4; 23; 33; 43; 53) ein Schmelzkleber ist.

6. Bekleidungsgegenstand oder Stoffstück (F), umfassend eine Applikation (9) nach Anspruch 1.

7. Verfahren zum Herstellen einer Applikation (9), umfassend die Schritte:
Bereitstellen eines Substrats (1; 12; 22; 32; 42; 52), umfassend Polyurethanmaterial und aufweisend eine erste Seite und eine zweite Seite, wobei das Substrat eine migrationsbeständige Barriere enthält;
Drucken einer Flock-Klebstoffschicht (2; 11; 21; 31; 41; 51) auf die erste Seite des Substrats;
Aufbringen einer Flock-Schicht (3; 10; 20; 30; 40; 50) in einem vorbestimmten mehrfarbigen Muster auf die Flock-Klebstoffschicht, wobei der Flock Fasern aufweist;
Fixieren der Flockfasern an der Flock-Klebstoffschicht;
Laminieren einer Klebstoffschicht (4; 23; 33; 43; 53) auf einer zweiten Seite des Substrats; und
Bereitstellen einer selektiv entfernbaren Trägerschicht (5; 13; 24; 44; 54), die eine Seite aufweist, die der zweiten Seite des Substrats und einer anderen Seite zugewandt ist,
wobei die Applikation gebildet wird, ohne dass Flock auf einen ablösbaren Klebstoff abgeschieden wird.

8. Verfahren nach Anspruch 7, enthaltend den Schritt zum Aufbringen der Klebstoffschicht auf ein Textil (F) .

## Revendications

1. Appliqué (9) pour appliquer un dessin sur un tissu, l'appliqué comprenant:
un substrat (1; 12; 22; 32; 42; 52) comprenant un matériau de polyuréthane, dans lequel le substrat comprend une barrière anti-migration;
un floc (3; 10; 20; 30; 40; 50) représentant un motif multicolore prédéterminé, le floc comprenant des fibres;
un adhésif de flocage (2; 11; 31; 41; 51) pour fixer les fibres de floc au substrat, l'adhésif de flocage étant imprimé sur le substrat;
un adhésif d'application (4; 23; 33; 43; 53), adjacent au substrat opposé aux fibres de floc, approprié pour coller l'appliqué à un tissu; et
une couche de support (5; 13; 24; 44; 54),
dans lequel le substrat, l'adhésif de flocage et l'adhésif d'application sont positionnés entre le floc et la couche de support, et
dans lequel l'appliqué est formé sans qu'un floc soit déposé sur un adhésive décollable.

2. Appliqué (9) selon la revendication 1, dans lequel le substrat (1; 12; 22; 32; 42; 52) présente de multiples couleurs, visibles à travers le floc (3; 10; 20; 30; 40; 50).

3. Appliqué (9) selon la revendication 1, dans lequel le substrat (1; 12; 22; 32; 42; 52) est un film.

4. Appliqué (9) selon la revendication 2, dans lequel le substrat est un motif holographique.

5. Appliqué (9) selon la revendication 1, dans lequel l'adhésif d'application (4; 23; 33; 43; 53) est thermofusible.

6. Vêtement ou pièce de tissu (F) comprenant un appliqué (9) selon la revendication 1.

7. Procédé de fabrication d'un appliqué (9), comprenant les étapes suivantes:
prévoir un substrat (1; 12; 22; 32; 42; 52) comprenant un matériau de polyuréthane et présentant un premier côté et un second côté, dans lequel le substrat comprend une barrière anti-migration;
imprimer une couche adhésive de floc (2; 11; 31; 41; 51) sur le premier côté du substrat;
appliquer une couche de floc (3; 10; 20; 30; 40 50) sous la forme d'un motif multicolore prédéterminé sur la couche adhésive de floc, le floc comprenant des fibres;
fixer les fibres de floc à la couche adhésive de floc;
stratifier une couche adhésive (4; 23; 33; 43; 53) sur un second côté du substrat; et
fournir une couche de support sélectivement amovible (5; 13; 24; 44; 54) qui présente un côté faisant face au second côté du substrat et un autre côté,
dans lequel l'appliqué est formé sans qu'un floc soit déposé sur un adhésive amovible.

8. Procédé selon la revendication 7, comprenant l'étape d'application de la couche adhésive à un textile (F).
